

## UNITED STATES PATENT OFFICE

2,159,926

## METHOD OF SOFTENING PLASTIC SHEETS

Julius F. T. Berliner, Wilmington, Del., assignor  
to E. I. du Pont de Nemours & Company, Wil-  
mington, Del., a corporation of Delaware

No Drawing. Application May 9, 1935,  
Serial No. 20,603

5 Claims. (Cl. 18—56)

This invention relates to solvent compositions and more particularly to new solvents for use in temporary softening of nitrocellulose plastics.

It is known that in the use of nitrocellulose plastics in covering operations, particularly in covering such objects as wood heels, toilet seats, hamper tops, high chair trays, and the like, it is necessary first to soften the plastic to a pliable condition such that it may be readily worked and fitted to the object to be covered. After softening of the plastic sheet it is easily stretched to cover the mold or the form desired, and upon drying, or evaporation of the softener, the material shrinks and, particularly when cement is used, clings tenaciously to the object covered. By nitrocellulose plastics I mean cellulose nitrates with which has been incorporated camphor and/or other plasticizing agents such as castor oil, tricresyl phosphate, diacetone and the like, or, generally, nitrocellulose-containing materials such as those of the types represented by materials known under the trade-marked names "Pyralin", "Celluloid", "Fibreloid", "Lucite", and the like.

Various solvents and mixtures of solvents have been proposed for the purpose of temporarily softening such materials, but due to the particular limitations as to only partial solvent effect, softening effect upon the plastic, and relatively high volatility, or evaporation rate after application, it has been found necessary in the past to use mixtures which have deleterious effects upon the operator. Thus, altho many materials have been proposed, up to the present invention, the solvent which has been found preferable has been an aqueous solution of methanol and acetone in which nitrocellulose plastics are softened but not dissolved. A non-aqueous solution of these materials completely rather than partially dis-  
solves the plastic. Altho this aqueous solution has been extensively used, representing as it does a softener which is satisfactory as to its softening effect and of fairly rapid evaporation rate, nevertheless it is characterized by several dis-  
tinct disadvantages. Thus, this solvent has an appreciable and deleterious effect upon the hands of the operator working with it, and as the operator customarily works for long periods with hands immersed, or partially immersed, in the solvent, the importance of the solvent's physical effect is appreciable. Furthermore, such methanol-acetone solutions dissolve out considerable quantities of camphor, which in turn necessitates the addition of camphor to the solvent so that the plastic may, after evaporation of the solvent,

have the same constitution as before treatment.

It is an object of this invention to overcome these and other disadvantages of the prior art and to produce a new and improved solvent.

Another object of the invention is to provide a new method of softening nitrocellulose plastics.

Other objects and advantages of the invention will be apparent by reference to the following specification in which its preferred embodiments and details are set forth.

According to this invention nitrocellulose plastics may be advantageously softened by use of a solution of methanol and higher ketones which are immiscible or at least only partly miscible with water. This softening solution may be used alone, altho I prefer, as is the case in the methanol-acetone solutions, to dilute the softener with water so that the final composition is constituted of from 3-4 parts by volume of methanol-higher ketone solution per part of water, preferably about 3.25 parts solvent per part of water.

The higher ketones which I have found to be so advantageous are those generally of from 4 to 9 carbon atoms per molecule and particularly those which are obtainable by the oxidation or dehydrogenation of the mixture of branched-chain secondary alcohols, obtainable by the catalytic pressure hydrogenation of oxide of carbon. Although mixtures of higher ketones generally and the complete mixture of ketones obtainable as above described are desirable and give superior results when mixed with methanol, I have found that best results are obtained by use of one or more of those ketones obtainable by oxidation or dehydrogenation of the branched-chain secondary alcohols obtainable as above described, or a mixture of them, which have boiling ranges between 115-128° C., namely, methyl isopropyl, ethyl isopropyl and diisopropyl ketones. The ketone, such as diisopropyl ketone, or the mixture of boiling point range 115-128° C. is mixed with methanol in the proportions of from about 9 to 25 parts, preferably about 13 parts, by volume ketone to about 75 to 91 parts, preferably about 87 parts, methanol. Preferably 3 1/4 parts of this solution is diluted with about one part of water before use.

Into such a solution is dipped a sheet of cellulose plastic which is softened therein for about 30 minutes. At the expiration of this soaking the completely pliable sheet is removed from the softening bath, cement applied to the form or mold to be covered, and then pressed firmly around the object. After about an hour the covering becomes hard and if left over night will be

found to be ready for use, the major part if not all of the solvent having evaporated.

The material of this invention has no deleterious effect upon the hands of the operator, has a lower evaporation rate, which is more satisfactory from an operating standpoint, and sustains its strength for a longer time than materials previously used extensively, and, since camphor is not appreciably soluble therein, obviates the necessity of adding camphor to the softener to keep stable the plasticizer content of the nitrocellulose being treated.

I have found that the softener of this invention is generally easier to use for covering operations and, at the same time that more satisfactory results are obtained, a lower ketone content (corresponding to the acetone in previously used softeners) is possible than with methanol-acetone solutions heretofore used in industry.

The composition of this invention may be used advantageously in all operations which involve temporary softening of nitrocellulose plastics for whatever purpose it is desired, but is particularly suited for leather belt compositing, production of nitrocellulose plastic novelties, for covering operations such as previously set forth, and the like, wherein, for a short time at least, such plastics must be pliable and workable.

By utilizing the softener of this invention nitrocellulose plastics are made as soft and pliable as wet chamois and can be easily stretched to fit and cemented to whatever form desired.

Cellulose nitrate sheeting softened by the material of this invention has a better body than obtained with other material shows little or no tendency to curl, takes a cleaner, sharper embossing, remains in workable condition for a longer time, has less tendency to crack or split after application to wood heels or the like, and, importantly, is wholly free from the toxic effect upon the operator which is such a disadvantageous characteristic of previous softening solutions. Furthermore, as an economical advantage, the material of this invention has a slower rate of evaporation than other softeners and is less inflammable.

Various changes may be made in the present invention without departing therefrom or sacrificing any of the advantages thereof.

I claim:

1. In plastic sheeting operations, the method of softening but not dissolving sheeting of nitrocellulose plastic compositions which comprises treating such compositions with a solution of

about one part by volume of water and 3 to 4 parts of a solution containing about 75 to 91 parts of methanol and about 9 to 25 parts of a relatively water-immiscible ketone of from 4 to 9 carbon atoms per molecule having a boiling point in the range of about 115-128° C. and obtainable by oxidation of the secondary branched chain aliphatic alcohols produced by the catalytic pressure hydrogenation of oxide of carbon.

2. In plastic sheeting operations, the method of softening but not dissolving sheeting of nitrocellulose plastic compositions which comprises treating such compositions with a solution of about one part by volume of water and 3 to 4 parts of a solution comprising about 87 parts of methanol and about 13 parts of a relatively water-immiscible ketone of from 4 to 9 carbon atoms per molecule, having a boiling point in the range of about 115-128° C., and obtainable by oxidation of the secondary branched chain aliphatic alcohols produced by the catalytic pressure hydrogenation of oxide of carbon.

3. In plastic sheeting operations, the method of softening but not dissolving sheeting of nitrocellulose plastic compositions which comprises treating such compositions with a solution of about one part by volume of water and 3 to 4 parts of a solution containing about 75 to 91 parts of methanol and about 9 to 25 parts of the mixture of methyl and ethyl isopropyl, and diisopropyl ketones obtainable by oxidation of the secondary branched chain aliphatic alcohols produced by the catalytic pressure hydrogenation of oxide of carbon.

4. In plastic sheeting operations, the method of softening but not dissolving sheeting of nitrocellulose plastic compositions which comprises treating such compositions with a solution of about one part by volume of water and 3 to 4 parts of methanol and about 13 parts of the mixture of methyl and ethyl isopropyl, and diisopropyl ketones obtainable by oxidation of the secondary branched chain aliphatic alcohols produced by the catalytic pressure hydrogenation of oxide of carbon.

5. In plastic sheeting operations, the method of softening but not dissolving sheeting of nitrocellulose plastic compositions which comprises treating such compositions with a solution of about one part by volume of water and 3 to 4 parts of a solution comprising about 87 parts of methanol and about 13 parts of diisopropyl ketone.

JULIUS F. T. BERLINER.